

# UNITED STATES PATENT OFFICE.

FEDERICO GIOLITTI, OF TURIN, ITALY, ASSIGNOR TO SOCIETÀ ANONIMA ITALIANA GIO, ANSALDO & C., OF GENOA, ITALY.

## PROCESS OF HEAT TREATMENT OF STEEL.

1,296,649.

Specification of Letters Patent.

Patented Mar. 11, 1919.

No Drawing.

Application filed October 14, 1914. Serial No. 866,702.

*To all whom it may concern:*

Be it known that I, FEDERICO GIOLITTI, a subject of the King of Italy, residing at No. 75 Stradale Moncalieri, in Turin, Italy, have 5 invented certain new and useful Improvements in Processes of Heat Treatment of Steel, of which the following is a specification.

This invention relates to an improved 10 heat treatment in the manufacture of any article of ingot or wrought steel and especially of gun parts and armor plates.

The object of this invention is to diminish 15 the brittleness of the material while increasing its strength and elongation under tensile stress, and its tenacity (that is, its power to resist shock).

The improved heat treatment is differentiated essentially from the other treatments 20 proposed hitherto, by the fact that in the known treatments the heating before hardening is effected at a single temperature, the value of which is determined by the latest point of transformation of the steel, where- 25 as according to the present improved process the heating for the hardening is effected successively at two different strictly determined temperatures, the passage from the first temperature to the second temperature being 30 gradually effected.

The temperatures above referred to are determined as follows:

1. The first temperature is comprised in the interval in which the diffusion phenomena of the different components in the structural elements of the steel occur with the greatest rapidity, without injuriously affecting the strength of the steel.

The steel under treatment must therefore 40 be heated to a temperature which is at least 100° C. higher than the third transformation point on heating of the steel in question.

As is well known, the said interval varies 45 in amplitude and position according to the composition of the steel; but it can be surely and easily determined by means of mechanical or micrographic tests or thermic analysis.

2. The second temperature is 30° C. lower 50 at least than the one which is employed for producing the ordinary homogeneous temper. This second temperature is slightly

greater, that is to say about 50° C. higher than that corresponding to the latest point of transformation to heat ( $Ar_3$ ) of the treated steel, but it is necessary in practice 55 to exceed this limit, more or less, according to the shape and dimensions of the manufactured articles and their composition.

An example of the mode of application of the improved treatment is the following: 60

The article to be treated (which may consist either of a rough rolled or rough wrought or a previously heat treated material) is first gradually heated in a suitable furnace until the entire mass of the article has reached the 65 aforesaid first temperature. This first temperature is maintained constant during an interval of time, experimentally determined, which may vary between very large limits according to the properties of the steel and 70 the shape and the dimensions of the treated articles. For a semi-hard carbon steel this interval may vary from one hour or less for pieces of 2-3 kg. or less to 20 hours or more for pieces of 10 tons or more. 75

The temperature of the furnace is next gradually changed to the aforesaid second temperature. This second temperature is maintained constant for a shorter interval of time than in the case of the first temperature or first heating. The article is 80

then quenched in cold or warm water or in oil, or is hardened by sprinkling. This treatment is generally followed by one of the ordinary tempering or re-heating (annealing) processes when a material with high tenacity and elongation is desired; or it may be followed by one of the well known tempering or hardening processes if it is intended to produce a material having a high 90

degree of hardness; or by one of the ordinary processes for producing a negative hardness (softening) of the articles having a heterogeneous composition, which results partly in a hard and partly in a tenacious 95 texture of the article after treatment.

To give a practical example for the treatment of a determined object formed of a determined steel we are now going to describe the following case:— 100

The object submitted to the thermic treatment forming the subject-matter of the pres-

ent application is a cylinder having a diameter of 50 centimeters and a length of 6 meters, made of cast steel of the following composition:—

|    |            |         |
|----|------------|---------|
| 5  | Carbon     | 0.25 %  |
|    | Manganese  | 0.40 %  |
|    | Silicon    | 0.10 %  |
|    | Sulfur     | 0.005 % |
| 10 | Phosphorus | 0.008 % |
|    | Nickel     | 2.56 %  |
|    | Chromium   | 0.55 %  |
|    | Vanadium   | 0.15 %  |
|    | Tungsten   | 0.78 %  |

15 The third transformation point on heating of a steel of this composition is in the neighborhood of 900° C., while the corresponding point on the cooling curve is between 20 580°-600° C.

From the tests made it appears that the best thermal treatment for this steel according to the principles of the processes subject-matter of the present application is 25 the following one:—

(1) Slow heating during about 18 hours up to a uniform temperature of 1070° C. throughout the whole mass of the piece.

(2) Maintaining the above said temperature of 1070° C. for six hours.

(3) Slow cooling (during about six hours) down to a uniform temperature of 680° C.

(4) Maintaining the above temperature of 680° C. for about six hours.

(5) Quenching in oil at ordinary temperature.

With a steel containing the constituents referred to in the proportions given below, the region in which the diffusion phenomena 40 occur with the greatest rapidity on heating will be found to be between 980 and 1050° C., and on cooling, in the neighborhood of 700°-750° C.

|    |            |         |
|----|------------|---------|
| 45 | Carbon     | 0.40 %  |
|    | Manganese  | 0.60 %  |
|    | Silicon    | 0.15 %  |
|    | Sulfur     | 0.009 % |
|    | Phosphorus | 0.02 %  |
| 50 | Chromium   | 2.20 %  |
|    | Nickel     | 2.50 %  |

A steel article, for example, a connecting

rod weighing 250 kgs., would be treated as follows:—

(a) Heated to 1000° C. during about 3 hours.

(b) Gradually cooled to 800° C. during an interval of 2 hours.

(c) Quenched in water from a temperature of 800° C.

With a carbon steel containing the constituents specified below in the proportion set forth:—

|    |            |         |
|----|------------|---------|
| 65 | Carbon     | 0.45 %  |
|    | Manganese  | 0.52 %  |
|    | Silicon    | 0.10 %  |
|    | Sulfur     | 0.05 %  |
|    | Phosphorus | 0.004 % |

70

the treatment would be effected as follows:—

(1) Heating gradually to a temperature of about 900° C.

(2) Maintaining the steel at this temperature for from 2 to 12 hours.

(3) Slow cooling to about 800° C.

(4) Maintaining the steel at this temperature for a period equal to one-half that stated under (1).

(5) Hardening in warm water or oil at the ordinary temperature.

(6) If necessary, tempering to obtain the desired tensile strength.

Having now described my invention, what I claim as new and desire to secure by Letters Patent is:—

The process of heat treatment of steel which comprises heating the steel to a temperature in the neighborhood of that at which the diffusion phenomena of the different components of the steel take place with the greatest rapidity, that is to say at least 100° C. higher than the third transformation point on heating of the steel under treatment, then lowering its temperature to at least 30° C. below the temperature necessary for effecting the ordinary uniform hardening and therefore at least about 50° C. above the critical point  $Ar_3$ .

In testimony whereof I have signed my name to this specification in the presence of two subscribing witnesses.

FEDERICO GIOLITTI

Witnesses:

GIACOMO CARDARA,

A. BORAGINO.